# EUROPEAN PATENT SPECIFICATION

(11) **EP 3 395 984 B1**
(45) Date of publication and mention of the grant of the patent: **29.01.2020**
(21) Application number: 16879157.2
(22) Date of filing: 03.11.2016
(51) Int. Cl.: C22C 38/12, C22C 38/08, C22C 38/04, C22C 38/02, C21D 8/02, C21D 9/50, C21D 1/25, C21D 6/00

(54) **STEEL SHEET HAVING EXCELLENT PWHT RESISTANCE FOR LOW-TEMPERATURE PRESSURE VESSEL AND METHOD FOR MANUFACTURING SAME**
STAHLBLECH MIT AUSGEZEICHNETER PWHT-BESTÄNDIGKEIT FÜR NIEDERTEMPERATURDRUCKBEHÄLTER UND VERFAHREN ZUR HERSTELLUNG
TÔLE D'ACIER PRÉSENTANT UNE EXCELLENTE RÉSISTANCE AU TRAITEMENT THERMIQUE APRÈS SOUDAGE POUR RÉCIPIENT SOUS PRESSION À BASSE TEMPÉRATURE ET SON PROCÉDÉ DE FABRICATION

(30) Priority: 22.12.2015 KR 20150183528
(43) Date of publication of application: 31.10.2018
(73) Proprietor: POSCO, Pohang-si, Gyeongsangbuk-do 37859 (KR)
(72) Inventor: HONG, Soon-Taik, Pohang-si, Gyeongsangbuk-do 37877 (KR)
(74) Representative: Potter Clarkson
(86) International application number: PCT/KR2016/012566
(87) International publication number: WO 2017/111290

(56) References cited:
- EP-A2- 2 520 680
- JP-A- S6 126 727
- JP-A- 2013 533 921
- JP-A- 2015 124 435
- KR-A- 20150 101 734
- KR-B1- 100 663 219
- KR-B1- 100 833 071
- KR-B1- 101 388 334

## Description

### [Technical Field]

The present disclosure relates to a thick steel plate used in a low-temperature pressure vessel, a ship, a storage tank, a structural steel, and the like, and a method for manufacturing the same, and more particularly, to a steel plate having excellent PWHT resistance and low-temperature toughness for a low-temperature pressure vessel in which a tensile strength is 600 MPa or more, and a method for manufacturing the same.

### [Background Art]

As a thick plate steel material having high strength for low-temperature uses, a mixed structure including ferrite, a martensite structure, and a bainite structure, or a nearly single-phase structure mainly consisting of bainite and ferrite, or the like, is widely known.

It is necessary to have high strength, since the steel material itself is usable as a structural material at the time of construction. Meanwhile, this high strength structural steel material is required to have excellent PWHT resistance. The high strength hot rolled steel material manufactured through a general normalizing treatment may have a mixed structure of ferrite and pearlite. However, when a PWHT treatment is performed in a subsequent process of a steel material having the structure, a carbide is formed along a grain boundary, and thus, strength and toughness of the steel material are lowered, failing to guarantee physical properties required for PWHT. An example of the conventional technique regarding this is disclosed in Korean Patent Laid-Open Publication No. 2012-0011289.

The Korean Patent Laid-Open Publication suggests a high strength steel material for LPG having a strength of 500 MPa or more including: in terms of wt%, 0.08-0.15% of C, 0.2-0.3% of Si, 0.5-1.2% of Mn, 0.01-0.02% of P, 0.004-0.006% of S, more than 0%-0.01% or less of Ti, 0.05-0.1% of Mo, 3.0-5.0% of Ni, and a balance of Fe and inevitable impurities, characterized in that Ni and Mo are added to the steel composition component.

However, since the invention disclosed in the above-described publication is a steel material manufactured through general normalizing, there is a problem in that deterioration of strength and toughness of the steel material after PWHT treatment is not avoidable even in the case that Ni, or the like, is added.

Therefore, in a thick steel plate having high strength used in a low-temperature pressure vessel, a ship, a storage tank, a structural steel, and the like, there is growing demand for development of a high strength steel material having excellent PWHT resistance for an extended period of time.

### [Related Art Document]

(Patent Document 1) Korean Patent Laid-Open Publication No. 2012-0011289

JP 2015 124435 A discloses a thick steel plate used for nuclear reactor containment vessels, comprising a microstructure containing lower bainite and tempered martensite.

JPS61 26727 A discloses a non-thermal refining type high strength steel having thick section and comprising carbon, silicon, manganese, nickel and soluble aluminium having a mixed structure consisting of over 60% martensite and over 5% bainite in any part of the whole structure.

### [Disclosure]

### [Technical Problem]

An aspect of the present disclosure is to provide a steel plate having excellent PWHT resistance for an extended period of time and high strength of a low-temperature pressure vessel by controlling a steel composition, and cooling and heat treatment processes to form a microstructure into a mixed structure of tempered bainite and tempered martensite, and a method for manufacturing the same.

However, technical problems to be achieved in the present disclosure are not limited to the above mentioned problems, and other non-mentioned problems will be clearly understood by those skilled in the art from the following descriptions.

### [Technical Solution]

According to an aspect of the present disclosure, a steel plate having excellent PWHT resistance for a low-temperature pressure vessel includes: in terms of wt%, 0.07-0.17% of C, 0.15-0.40% of Si, 0.3-0.7% of Mn, 0.012% or less of P, 0.015% or less of S, 3.0-4.0% of Ni, 0.03-0.25% of W, and a balance of Fe and inevitable impurities, wherein the steel plate has a microstructure including 25-80 area% of tempered bainite and a balance of tempered martensite.

The steel plate maintains tensile strength at 600 MPa or more even when the steel plate is subjected to PWHT for a maximum of 20 hours at 580-640°C.

The steel plate may have a Charpy impact energy value of 200J or more at -110°C even when the steel plate is subjected to PWHT for a maximum of 20 hours at 580-640°C.

According to another aspect of the present disclosure, a method for manufacturing a steel plate having excellent PWHT resistance for a low-temperature pressure vessel includes:
reheating a steel slab at a temperature of 1050-1250°C, the steel slab including, in terms of wt%, 0.07-0.17% of C, 0.15-0.40% of Si, 0.3-0.7% of Mn, 0.012% or less of P, 0.015% or less of S, 3.0-4.0% of Ni, 0.03-0.25% of W, and a balance of Fe and inevitable impurities;
hot rolling the reheated steel slab and terminating the rolling at a temperature of 800°C or more to obtain a hot rolled steel plate;
heating the hot rolled steel plate to 800-950°C, followed by water cooling at a cooling rate of 2.5-30°C/sec; and
tempering the water cooled steel plate at 550-660°C for (1.5×t + (10) minutes to (1.5xt + 30) minutes [wherein t is a thickness (mm) of the steel material].

The method may further include: a PWHT process for a maximum of 20 hours at 580-640°C after the tempering.

A steel microstructure obtained by the tempering may have 25-80 area fraction % of tempered bainite and a balance of tempered martensite.

### [Advantageous Effects]

As set forth above, according to an exemplary embodiment in the present disclosure, a steel plate having excellent PWHT resistance for a low-temperature pressure vessel, stably usable at a low temperature of about -110°C while satisfying a tensile strength of 600 MPa or more, may be effective provided.

### [Best Mode for Invention]

Hereinafter, the present disclosure will be described in detail.

First, a steel plate having excellent PWHT resistance for a low-temperature pressure vessel of the present disclosure is described.

The steel plate of the present disclosure includes, in terms of wt%, 0.07-0.17% of C, 0.15-0.40% of Si, 0.3-0.7% of Mn, 0.012% or less of P, 0.015% or less of S, 3.0-4.0% of Ni, 0.03-0.25% of W, and a balance of Fe and inevitable impurities, and specific steel composition components and reasons for limiting the components are as follows.

In the present disclosure, C is limited to a content of 0.07-0.17%. When the content is less than 0.07%, a self-strength of a matrix may be deteriorated. When the content is more than 0.17%, weldability of the steel plate may be greatly deteriorated.

Si is a component to be added for a deoxidation effect, a solid-solution strengthening effect and an impact transition temperature increasing effect, and is added in a content of 0.15% or more in order to achieve these additive effects. However, when the content of Si is more than 0.40%, the weldability is lowered and an oxide film is excessively formed on a surface of the steel plate, such that the content thereof is limited to 0.15-0.40%.

Mn forms MnS, a non-metallic inclusion elongated together with S, to lower a room temperature elongation and a low-temperature toughness, such that a content of Mn is controlled to be 0.7% or less. However, due to characteristics of the components of the present disclosure, when the content of Mn is less than 0.3%, it is difficult to ensure adequate strength, such that an added content of Mn is limited to 0.3-0.7%.

P is an element that deteriorates low-temperature toughness, such that a content of P is preferably suppressed as much as possible. However, since excessive cost is required to remove P in a steelmaking process, the content of P may be controlled within a range of 0.012% or less.

S is also an element that adversely affects low-temperature toughness together with P, but as similar to P, excessive cost may be required to remove S in a steelmaking process, such that the content of S may be controlled within a range of 0.015% or less.

Ni is the most effective element for improving low-temperature toughness. However, when an added content of Ni is less than 3.0%, low-temperature toughness may be deteriorated. When the added content is more than 4.0%, production cost may be increased. Therefore, Ni is added within a range of 3.0 to 4.0%.

In the present disclosure, W is an important element that is solid-solutionized in austenite to increase curing ability of austenite and precipitates into a carbide (W₂C) matched with a matrix to increase a strength of the steel. When W is added in a content of less than 0.03%, an addition effect may not be expected. When W is added in a content of more than 0.25%, a coarse precipitate may be formed during a casting process to deteriorate low-temperature toughness, such that the content of W is limited to 0.03-0.25%.

Meanwhile, the steel plate of the present disclosure may have a microstructure including 25-80 area% of tempered bainite and a balance of tempered martensite. When a fraction of the tempered bainite is less than 25%, an amount of the tempered martensite may be excessive, and low-temperature toughness of the steel plate may be deteriorated. On the other hand, when the fraction of the tempered bainite is more than 80%, it may be difficult to secure desired strength of the steel plate.

More preferably, the microstructure may include 30-70 area fraction% of tempered bainite and a balance of tempered martensite.

The steel plate having the above-described steel composition components and microstructure may effectively maintain tensile strength at 600 MPa or more and have excellent low-temperature toughness even when the steel plate is subjected to PWHT for a maximum of 20 hours at 580-640°C.

Next, a method for manufacturing a steel plate having excellent PWHT resistance for a low-temperature pressure vessel of the present disclosure will be described.

The method for the steel plate of the present disclosure includes: reheating a steel slab having the above-described steel composition components at 1050-1250°C; hot rolling the reheated steel slab and terminating the rolling at a temperature of 800°C or more to obtain a hot rolled steel plate; heating the hot rolled steel plate to 800-950°C, followed by water cooling at a cooling rate of 2.5-30°C/sec; and tempering the water cooled steel material at 550-660°C for {1.5×t + (10-30) } minutes [wherein t is a thickness (mm) of the steel material] .

First, in the present disclosure, the steel slab having the steel composition component is reheated at 1050-1250°C. When a reheating temperature is less than 1050°C, a solute atom may be difficult to be solid-solutionized, and when the reheating temperature is more than 1250°C, an austenite crystal grain size may be excessively coarse to lower physical properties of the steel plate.

Subsequently, in the present disclosure, the reheated steel slab is hot rolled. Specifically, in the present disclosure, the reheated steel slab is hot rolled, and the rolling is terminated at a temperature of 800°C or more. When a hot rolling temperature is less than 800°C, hot deformation resistance may increase at the time of rolling, which may result in a load on a rolling mill.

A reduction rate per pass in the hot rolling is preferably 5-30%.

In addition, in the present disclosure, the hot rolled steel plate is heated at 800-950°C and then water cooled at a cooling rate of 2.5-30°C/sec.

When a heating temperature is less than 800°C, an alloy component may be difficult to be sufficiently solid-solutionized, and when the heating temperature is more than 950°C, crystal grains may be coarsened, such that the toughness may be deteriorated.

In addition, when the cooling rate is less than 2.5°C/sec, the martensite structure may not be obtained. On the other hand, when the cooling rate is more than 30°C/sec, since a large amount of cooling water may be required, there is an economic burden of requiring additional cooling equipment, such that the cooling rate is limited to 2.5-30°C/sec.

Subsequently, in the present disclosure, the water cooled steel plate may be tempered.

Specifically, in the present disclosure, the water cooled steel plate may be tempered at 550-660°C for {1.5×t + (10-30) } minutes [wherein t is a thickness (mm) of the steel material] . When a tempering temperature is less than 550°C, the toughness may be deteriorated by excessive strength. When the tempering temperature is more than 660°C, strength may be excessively deteriorated.

Further, in the present disclosure, a tempering time may be determined to {1.5×t + (10-30)} minutes [wherein t is a thickness (mm) of the steel material], and a specific reason for the limitation is as follows.

In other words, when the tempering time is shorter than the above criteria, the tempered martensite structure may be difficult to be obtained. On the other hand, when the tempering time is longer than the above criteria, overall productivity may be damaged.

By the tempering heat treatment under the above-described condition, the steel microstructure including 25-80 area% of tempered bainite and a balance of tempered martensite may be obtained.

More preferably, the microstructure may include 30-70 area fraction% of tempered bainite and a balance of tempered martensite.

Subsequently, in the present disclosure, PWHT heat treatment may be performed on the tempered steel plate to remove stress of a welded portion after welding for manufacturing a pressure vessel. In other words, a PWHT process for a maximum of 20 hours at 580-640°C may be further included.

When a PWHT temperature is less than 580°C, it may be difficult to remove residual stress from the welded portion, or the like, and when the PWHT temperature is more than 640°C, strength of the steel material may be significantly lowered. Further, when the PWHT time is more than 20 hours, strength may be excessively deteriorated.

### [Mode for Invention]

Hereinafter, the present disclosure will be described in more detail through Examples.

Steel slabs having composition components shown in Table 1 below were prepared, respectively, and these steel slabs were reheated at 1100°C. Then, the reheated steel slabs were hot rolled at a reduction rate of 15% per pass, and the hot rolling was terminated at 900°C to manufacture hot rolled steel plates having a predetermined thickness.

The hot rolled steel plates were heated at an austenitization temperature and water cooled under conditions shown in Table 2 below, and subsequently, tempered at temperature and time shown in Table 2 below. In addition, the tempered steel plates were also subjected to PWHT treatment under the conditions shown in Table 2 below.

As described above, the PWHT-treated steel plates were evaluated for yield strength, tensile strength and low temperature toughness, and results thereof are also shown in Table 2 below. Meanwhile, in Table 2 below, the low temperature toughness is a result of evaluating a specimen having V notch at -110°C with the Charpy impact energy value obtained by performing the Charpy impact test.

**[Table 1]**

| Kind of steel | Composition component (wt%) | | | | | | |
|---|---|---|---|---|---|---|---|
| | C | Mn | Si | P | S | Ni | W |
| Inventive steel a | 0.10 | 0.62 | 0.29 | 0.009 | 0.0012 | 3.49 | 0.08 |
| Inventive steel b | 0.09 | 0.60 | 0.27 | 0.008 | 0.0010 | 3.45 | 0.11 |
| Inventive steel c | 0.10 | 0.65 | 0.28 | 0.010 | 0.0011 | 3.55 | 0.18 |
| Comparative steel d | 0.11 | 0.68 | 0.29 | 0.012 | 0.0012 | 3.50 | - |

**[Table 2]**

| Classification | Kind of steel | Heating temperature (°C) | Water cooling rate (°C/s ) | Tempering temperature (°C) | Tempering time (min) | PWHT temperature (°C) | PWHT time (hr) | Tempered bainite area fraction (%) | YS (Mpa) | TS (Mpa) | -11 0°C Impact toughness (J) |
|---|---|---|---|---|---|---|---|---|---|---|---|
| Inventive Example 1 | a | 850 | 15.0 | 650 | 50 | 630 | 15 | 60 | 568 | 608 | 256 |
| Inventive Example 2 | | 860 | 8.5 | 650 | 90 | 630 | 20 | 55 | 557 | 602 | 251 |
| Inventive Example 3 | b | 850 | 15.0 | 650 | 50 | 630 | 15 | 53 | 558 | 610 | 227 |
| Inventive Example 4 | | 860 | 8.5 | 650 | 90 | 630 | 20 | 50 | 557 | 605 | 233 |
| Inventive Example 5 | c | 850 | 15.0 | 650 | 50 | 630 | 15 | 48 | 560 | 615 | 230 |
| Inventive Example 6 | | 850 | 8.5 | 650 | 90 | 630 | 20 | 45 | 551 | 610 | 215 |
| Comparative Example 1 | D | 850 | Air cooling | 650 | 50 | 630 | 15 | 0 | 458 | 523 | 155 |
| Comparative Example 2 | | 850 | Air cooling | 650 | 90 | 630 | 20 | 0 | 442 | 516 | 148 |

As shown in Tables 1 and 2, it could be appreciated that in Inventive Examples 1-6 in which the steel composition components and the manufacturing process conditions satisfy the range of the present disclosure, after tempering treatment, the structure including 25-80 area fraction% of tempered bainite and a balance of tempered martensite could be obtained, such that as compared to Comparative Examples, yield strength and tensile strength after the subsequent PWHT were higher by about 100 MPa and 80 MPa, respectively, and -110°C low temperature toughness was also higher by 70J or more.

On the other hand, since the comparative steel d did not contain W, strength of the steel was relatively low. In Comparative Examples 1 and 2, since water cooling was not performed but air cooling was performed, the tempered bainite was not generated, such that the yield strength and tensile strength after the subsequent PWHT were lower than those of the Inventive Example, and the -110°C low temperature toughness was also lower than that of the Inventive Example.

## Claims

1. A steel plate having excellent PWHT resistance for a low-temperature pressure vessel comprising:
in terms of wt%, 0.07-0.17% of C, 0.15-0.40% of Si, 0.3-0.7% of Mn, 0.012% or less of P, 0.015% or less of S, 3.0-4.0% of Ni, 0.03-0.25% of W, and a balance of Fe and inevitable impurities,
wherein the steel plate has a steel microstructure including 25-80 area% of tempered bainite and a balance of tempered martensite, and
wherein the steel plate maintains tensile strength at 600 MPa or more even when the steel plate is subjected to PWHT for a maximum of 20 hours at 580-640°C.

2. The steel plate of claim 1, wherein the steel microstructure includes 30-70 area% of tempered bainite and a balance of tempered martensite.

3. The steel plate of claim 1, wherein the steel plate has a Charpy impact energy value of 200J or more at -110°C even when the steel plate is subjected to PWHT for a maximum of 20 hours at 580-640°C.

4. A method for manufacturing a steel plate having excellent PWHT resistance for a low-temperature pressure vessel, the method comprising:
reheating a steel slab at a temperature of 1050-1250°C, the steel slab including, in terms of wt%, 0.07-0.17% of C, 0.15-0.40% of Si, 0.3-0.7% of Mn, 0.012% or less of P, 0.015% or less of S, 3.0-4.0% of Ni, 0.03-0.25% of W, and a balance of Fe and inevitable impurities;
hot rolling the reheated steel slab and terminating the rolling at a temperature of 800°C or more to obtain a hot rolled steel plate;
heating the hot rolled steel plate to 800-950°C, followed by water cooling; and
tempering the water cooled steel material at 550-660°C for (1.5×t + (10) minutes to (1.5xt + 30) minutes [wherein t is a thickness (mm) of the steel material], and
wherein a cooling rate in the water cooling is 2.5 to 30°C/sec.

5. The method of claim 4, further comprising:
a PWHT process for a maximum of 20 hours at 580-640°C after the tempering.

6. The method of claim 4, wherein a microstructure of the tempered steel has 25-80 area% of tempered bainite and a balance of tempered martensite.

7. The method of claim 4, wherein a microstructure of the tempered steel has 30-70 area% of tempered bainite and a balance of tempered martensite.

8. The method of claim 4, wherein a reduction rate per pass in the hot rolling is 5-30%.

## Patentansprüche

1. Stahlplatte mit ausgezeichneter PWHT-Beständigkeit für einen Niedertemperaturdruckbehälter, umfassend:
in Gew.-%, 0,07-0,17 % C, 0,15-0,40 % Si, 0,3-0,7 % Mn, höchstens 0,012 % P, höchstens 0,015 % S, 3,0-4,0 % Ni, 0,03-0,25 % W und einen Rest Fe sowie unvermeidbare Verunreinigungen, wobei die Stahlplatte eine Stahlmikrostruktur aufweist, die 25-80 Flächen-% getempertes Bainit und einen Rest getempertes Martensit beinhaltet, und wobei die Stahlplatte eine Zugfestigkeit von 600 MPa oder mehr beibehält, selbst wenn die Stahlplatte maximal 20 Stunden lang bei 580-640 °C einer PWHT ausgesetzt wird.

2. Stahlplatte nach Anspruch 1, wobei die Stahlmikrostruktur 30-70 Flächen-% getempertes Bainit und einen Rest getempertes Martensit beinhaltet.

3. Stahlplatte nach Anspruch 1, wobei die Stahlplatte mit einem Charpy-Kerbschlagenergiewert 200 J oder mehr bei -110 °C aufweist, selbst wenn die Stahlplatte höchstens 20 Stunden lang bei 580-640 °C einer PWHT ausgesetzt wird.

4. Verfahren zum Herstellen einer Stahlplatte mit ausgezeichneter PWHT-Beständigkeit für einen Niedertemperaturdruckbehälter, wobei das Verfahren umfasst:
Wiedererhitzen einer Stahlbramme bei einer Temperatur von 1050-1250 °C, wobei die Stahlbramme in Gew.-% 0,07-0,17 % C, 0,15-0,40 % Si, 0,3-0,7 % Mn, höchstens 0,012 % P, höchstens 0,015 % S, 3,0-4,0 % Ni, 0,03-0,25 % W und einen Rest Fe sowie unvermeidliche Verunreinigungen beinhaltet;
Warmwalzen der wiedererhitzten Stahlbramme und Beenden des Walzens bei einer Temperatur von 800 °C oder mehr, um ein warmgewalztes Stahlblech zu erhalten;
Erhitzen der warmgewalzten Stahlplatte auf 800-950 °C, gefolgt von Wasserkühlung; und
Tempern des wassergekühlten Stahlmaterials bei 550-660 °C für (1,5 × t + (10) Minuten bis (1,5 × t + 30) Minuten [wobei t eine Dicke (mm) des Stahlmaterials ist] und wobei eine Abkühlgeschwindigkeit der Wasserkühlung 2,5 bis 30 °C/s beträgt.

5. Verfahren nach Anspruch 4, ferner umfassend:
einen PWHT-Vorgang für maximal 20 Stunden bei 580-640 °C nach dem Tempern.

6. Verfahren nach Anspruch 4, wobei eine Mikrostruktur des getemperten Stahls 25-80 Flächen-% getempertes Bainit und einen Rest getempertes Martensit aufweist.

7. Verfahren nach Anspruch 4, wobei eine Mikrostruktur des getemperten Stahls 30-70 Flächen-% getempertes Bainit und einen Rest getempertes Martensit aufweist.

8. Verfahren nach Anspruch 4, wobei eine Reduktionsrate pro Durchgang in dem Warmwalzen 5-30 % beträgt.

## Revendications

1. Plaque en acier ayant une excellente résistance à un traitement thermique post-soudage (PWHT), pour un récipient sous pression à basse température, comprenant :
0,07 à 0,17 % en poids de C, 0,15 à 0,40 % en poids de Si, 0,3 à 0,7 % en poids de Mn, 0,012 % en poids ou moins de P, 0,015 % en poids ou moins de S, 3,0 % à 4,0 % en poids de Ni, 0,03 à 0,25 % en poids de W et un reste constitué de Fe et d'impuretés inévitables,
dans laquelle la plaque d'acier a une microstructure en acier comprenant 25 à 80 % en surface de bainite trempée et un reste de martensite trempée, et
dans laquelle la plaque d'acier conserve une résistance à la traction de 600 MPa ou plus même lorsque la plaque d'acier est soumise à un PWHT pendant 20 heures au maximum, à une température de 580 à 640 °C.

2. Plaque en acier selon la revendication 1, dans laquelle la microstructure en acier comprend 30 à 70 % en surface de bainite trempée et un reste de martensite trempée.

3. Plaque en acier selon la revendication 1, dans laquelle la plaque en acier a une valeur d'énergie d'impact de Charpy de 200 J ou plus à -110 °C même lorsque la plaque en acier est soumise à un PWHT pendant 20 heures au maximum, à une température de 580 à 640 °C.

4. Procédé de fabrication d'une plaque en acier ayant une excellente résistance à un PWHT, pour un récipient sous pression à basse température, le procédé comprenant :
le réchauffement d'une brame en acier à une température de 1050 à 1250 °C, la brame en acier comportant, 0,07 à 0,17 % en poids de C, 0,15 à 0,40 % en poids de Si, 0,3 à 0,7 % en poids de Mn, 0,012 % en poids ou moins de P, 0,015 % en poids ou moins de S, 3,0 à 4,0 % en poids de Ni, 0,03 à 0,25 % en poids de W et un reste constitué de Fe et d'impuretés inévitables ;
le laminage à chaud de la brame en acier réchauffée et l'arrêt du laminage à une température de 800 °C ou plus, de façon à obtenir une plaque en acier laminée à chaud ;
le chauffage de la plaque en acier laminée à chaud à une température de 800 à 950 °C, suivi d'un refroidissement à l'eau ; et
le trempage du matériau en acier refroidi à l'eau à une température de 550 à 660 °C pendant (1,5 × t + 10) minutes à (1,5 × t + 30) minutes [t étant une épaisseur (mm) du matériau en acier], et le taux de refroidissement dans l'eau de refroidissement étant compris entre 2,5 et 30 °C/s.

5. Procédé selon la revendication 4, comprenant en outre :
un processus PWHT pendant 20 heures au maximum à une température de 580 à 640 °C après le trempage.

6. Procédé selon la revendication 4, dans lequel une microstructure de l'acier trempé présente 25 à 80 % en surface de bainite trempée et un reste de martensite trempée.

7. Procédé selon la revendication 4, dans lequel une microstructure de l'acier trempé présente 30 à 70 % en surface de bainite trempée et un reste de martensite trempée.

8. Procédé selon la revendication 4, dans lequel un taux de réduction par passage dans le laminage à chaud est compris entre 5 et 30 %.
